

## UNITED STATES PATENT OFFICE

2,041,131

## PROCESS FOR THE PREPARATION OF METALLIC BERYLLIUM BY ELECTROLYSIS

Gustav Jaeger, Neu-Isenburg in Hesse,  
GermanyNo Drawing. Application July 9, 1934, Serial No.  
734,414. In Germany July 10, 1933

4 Claims. (Cl. 204—19)

The object of my invention is a process for the preparation of pure beryllium metal by electrolysis.

It has been known before to prepare beryllium metal from beryllium chloride by electrolysis in which electrolysis a mixture of beryllium chloride and sodium chloride is utilized as electrolyte. This electrolysis has always been carried out with a great excess of sodium chloride. In consequence of the high melting point of the sodium chloride the temperature of the electrolyte had to be kept at a range of about 730 to 820° C. All the prescriptions therefore give an average temperature of 800° which corresponds approximately to the fusion point of sodium chloride. Since beryllium chloride, however, fuses already at 405° C.—as is well known—its vapor tension at a bath temperature of 800° is a very high one. Therefore very considerable quantities vaporize already which either get lost or have to be recovered in a rather complicated device.

According to my invention I carry out the electrolysis of the beryllium chloride by using a mixture of beryllium chloride and alkali metal chloride the fusion point of which is below 450° centigrade, and effecting the electrolysis at temperatures of 450° centigrade and lower.

Mixtures of beryllium chloride and alkali metal chloride which melt below 450° centigrade contain, as has been ascertained, a minimum of 30 percent beryllium chloride. The contents of the bath mixture as regards beryllium chloride may be raised considerably. The upper limit for increasing the contents as regards beryllium chloride in the electrolyte is given by the fact that pure beryllium chloride itself is a very bad conductor of the electric current or none at all. For this reason one is compelled to add to the beryllium chloride certain quantities of conducting salts. As such I use alkali metal chlorides. With great advantage I have used for the electrolysis mixtures which contain about 40 to 60 percent beryllium chloride whilst the rest consists of alkali metal chloride for instance sodium chloride or potassium chloride. Such mixtures may have a melting point as low as 350° C. In some cases a mixture of both these salts may be used. When using a mixture consisting of about 50 parts of beryllium chloride and 50 parts of sodium chloride the most favorable temperature

for carrying out the electrolysis was found to be 370 to 380° centigrade.

The process according to my invention offers advantage in various directions. The fact that the electrolysis is carried out at a comparatively low temperature—which in itself is already a great advantage—causes the loss of beryllium chloride by vaporization to be reduced to a minimum. Furthermore, at this temperature the melt is completely indifferent towards the material forming the vessel of the electric bath, and its viscosity is a very low one. The process of my invention works with excellent current yields which amount to as high as nearly 100 percent.

The beryllium metal which is obtained by working according to my invention is deposited in solid flakes which are exceedingly pure so that they may be fused to a regulus without any difficulty for instance in a current of hydrogen or nitrogen. Losses are practically avoided when working in accordance with my invention which on the other hand always occur when the metal is deposited in a pulverulent or gritty condition.

What I claim is:

1. A process for the preparation of beryllium metal by electrolysis from a mixture of beryllium chloride and alkali metal chloride which comprises using as electrolyte a mixture containing 50 parts of sodium chloride and 50 parts of beryllium chloride and electrolyzing at a bath temperature of between 370 to 380° centigrade.

2. A process for the preparation of beryllium metal which consists in electrolyzing at a temperature of between 350° C. and 450° C. a fused mixture of beryllium chloride and alkali metal chloride containing at least 30% of beryllium chloride.

3. A process for the preparation of beryllium metal which consists in electrolyzing at a temperature of between 370° C. and 380° C. a fused mixture of beryllium chloride and alkali metal chloride containing at least 30% of beryllium chloride.

4. A process for the preparation of beryllium metal which consists in electrolyzing at a temperature below 450° C. a fused mixture of beryllium chloride and alkali metal chloride containing from 40% to 60% of beryllium chloride.